

## UNITED STATES PATENT OFFICE.

JENS HERMAN CHRISTENSEN, OF COPENHAGEN, DENMARK.

## PROCESS OF MAKING MATCHES.

SPECIFICATION forming part of Letters Patent No. 786,629, dated April 4, 1905.

Application filed July 10, 1903. Serial No. 164,991.

*To all whom it may concern:*

Be it known that I, JENS HERMAN CHRISTENSEN, of 12 St. Kannikestraede, Copenhagen, in the Kingdom of Denmark, have invented 5 certain new and useful Improvements in Processes of Making Matches, of which the following is a specification.

The object of this invention is to provide a process by which headless matches of a durable 10 character and capable of easy ignition are produced.

For this purpose the invention consists in the process hereinafter described of making matches, which comprises the steps of nitrating 15 the match-sticks and then impregnating said nitrated sticks with an igniting composition.

In carrying out my new process the match-sticks, which are customarily of wood, are first 20 nitrated. This nitrating may be effected by submerging the tips of the sticks in a solution of nitric acid of any suitable degree of concentration. To the solution may be added other 25 substances which do not affect the desired action, but which serve for other purposes in connection with the nitrating. Nitric acid of about thirty per cent. is employed at the temperature at which no obnoxious formation of fumes takes place. This temperature is about 30 85° centigrade. The tips of the sticks are retained in the nitrating fluid until thoroughly impregnated. The completion of the treatment is indicated when the nitrated portion, which is at first red, becomes yellow. The 35 excess of nitric acid in the tips, which would subsequently become injurious owing to the hydrochloric acid being liberated in the igniting composition, may be removed or neutralized by simply washing the match-sticks in 40 hot water. The excess of acid may also be neutralized or rendered harmless by washing the sticks in an aqueous solution of suitable basic compounds or salts of weak acids which do not impart to the match-sticks hygroscopic 45 properties. In most cases it is preferable to use compounds of potassium, strontium, barium, or lead—for instance, hydrosulfid of ba-

rium. After the nitration the match-sticks are at their tips dipped into an igniting composition. Such a composition may, for instance, 50 consist of one hundred parts chlorate of barium with either four parts of nitrate of lead and six parts of chlorate of potassium, or eight parts nitrate of copper and four parts chlorate of potassium, or with only five parts of 55 hydrosulfid of barium, together with the quantities of water necessary for dissolving the above-mentioned substance at boiling temperature. This composition is of itself non-explosive. In combination with wood it inflames under the heat of friction. Such combination is promoted by the nitration of the 60 match-sticks. The tips are retained in this composition for a period of two or three minutes. They are then removed and permitted 65 to dry. When dried, the matches are ready for the boxes.

Instead of removing or neutralizing the excess of nitric acid before dipping the tips into the igniting solution these two steps may be 70 carried out simultaneously by adding to the igniting composition a suitable neutralizing substance or a salt of the above-mentioned weak acids. Simultaneously with the removal of the excess of nitric acid qualities may be 75 imparted to the matches which increase their inflammability. Thus, for example, sulfur may be added by employing as a neutralizing agent a solution containing hydrosulfid of barium or other easily-inflammable organic compounds or by employing the salt of a weak 80 organic acid.

The matches produced by my new process are extremely durable, ignite easily, and are provided with soft tips. The nitration acts 85 to soften the tips. They are very easily ignited and owing to the softness of the tips do not injure the surface across which they are drawn for ignition.

Having thus described my invention, I claim 90 as new and desire to secure by Letters Patent—

1. The herein-described process of making matches, which consists in subjecting the tips of match-sticks to the action of a nitrating

composition, removing the excess of nitric acid and then impregnating the sticks with an igniting composition.

2. The herein-described process of making 5 matches, which consists in nitrating match-sticks, washing the nitrated sticks and then impregnating the same with an igniting composition containing salts of a weak acid.

In testimony that I claim the foregoing as my invention I have signed my name in presence of two subscribing witnesses.

JENS HERMAN CHRISTENSEN.

Witnesses:

A. COFFMAN-BANG,  
J. C. JACOBSEN.